

# UNITED STATES PATENT OFFICE.

AUGUST SIEGMUND, OF LUDWIGSHAFEN, GERMANY, ASSIGNOR TO THE  
BADISCHE ANILIN AND SODA FABRIK, OF SAME PLACE.

## PROCESS OF DYEING.

SPECIFICATION forming part of Letters Patent No. 659,556, dated October 9, 1900.

Application filed July 24, 1900. Serial No. 24,712. (No specimens.)

*To all whom it may concern:*

Be it known that I, AUGUST SIEGMUND, 5  
dyer, a subject of the King of Prussia, German  
Emperor, residing at Ludwigshafen-on-  
the-Rhine, in the Kingdom of Bavaria and  
Empire of Germany, have invented new and  
useful Improvements in Processes of Dyeing  
Wool, of which the following is a specification.

In the art of wool-dyeing it is often very  
desirable to combine perfect level dyeing with  
the highest possible clearness and brilliancy  
of shade attainable, especially where delicate  
shades are demanded. This is particularly  
true in the case of zephyr yarns. It has long  
been known that no matter how carefully the  
wool has been bleached prior to dyeing the  
shade obtained is always more or less sad.  
This sad appearance can be removed only by  
the old and well-known operation of stoving—  
that is, by subjecting the dyed and whizzed  
goods, whether loose, spun, or woven, to a  
treatment with sulfur dioxide in the sulfur-  
chamber. The stoving operation is absolutely  
essential for certain dyestuffs when used  
where the highest possible brilliancy is re-  
quired, and without such treatment many  
dyestuffs would be inapplicable to this branch  
of the art of dyeing—for example, rhodamin,  
auramin, &c. It is obvious that only such  
dyestuffs are available for this purpose as are  
fast against sulfur dioxide and which are con-  
sequently known in the art as being “fast to  
stoving.” It is also obvious that this stoving  
operation increases the time necessary for the  
dyeing of a certain quantity of material and  
also adds to the cost of manufacture of the  
dyed goods. Moreover, this old process is at-  
tended with an expenditure of a very great  
amount of care, brought about by the diffi-  
culty it causes in dyeing to shade, inasmuch  
as it frequently causes a change in shade or  
a lightening or both, which is exceedingly  
troublesome and irksome to rectify and so  
causes an extra expenditure of labor and dye-  
stuff. The rectification of such a shade is an  
operation not generally attended with suc-  
cess.

The object of this invention is to obviate  
this additional and irksome operation of stov-  
ing and the attendant labor of bringing the  
stoved goods to shade, and thus to simplify

and to reduce the cost of the process of ob-  
taining these highly-desirable level and clear  
shades.

This invention is based upon the new and 55  
striking observation that all the advantages  
which dyed goods show after having been sub-  
jected to stoving are obtained by adding to  
the dye-bath simultaneously with the dyestuff  
and chemicals sulfurous acid or such sub- 60  
stances as will develop sulfurous acid under  
the conditions prevailing in the dye-bath,  
dyeing, and finishing, as usual, without stov-  
ing. It has also been observed that there is  
a decided gain in clearness of shade as well 65  
as also a saving in the amount of dyestuff  
required to produce a certain shade as against  
the old process. In addition to this there is  
also in many cases the great advantage that  
the dyer can dye to shade directly and with- 70  
out running the risk of being obliged to sub-  
mit the stoved goods to a subsequent and  
troublesome treatment with dyestuff in order  
to get to shade. These effects and advan-  
tages are not to be obtained by subjecting the 75  
dyed goods to a bath of sulfurous acid, whether  
the sulfurous acid be added to the dye-bath  
after it has been exhausted or whether the  
dyed goods are treated in the well-known way  
in a separate bath containing sulfurous acid, 80  
or in that case a lightening of the shade with-  
out any increase in brilliancy results—that  
is, the dyestuff is stripped from off the fiber.

In the following an example is given as to  
how this invention can be applied. For one 85  
hundred pounds of goods prepare a dye-bath  
as follows: three hundred and seventy-five  
(375) gallons of water, five (5) pounds of bi-  
sulfite of soda of 38° Baumé, three and a  
quarter (3 $\frac{1}{4}$ ) ounces of rhodamin 3B, ten (10) 90  
pounds of Glauber salts, and two (2) pounds  
of sulfuric acid of 66° Baumé; enter, bring to  
boil, and dye to shade.

In place of the rhodamin in the preceding  
example any of the other dyestuffs which 95  
are fast to stoving may be used. Among  
these may be particularly mentioned auras-  
min, methyl violet, victoria blue, palatin scar-  
let, fast yellow, acid violet 4R, alkali violet,  
victoria night-blue, &c.

What I claim is—

1. The process of dyeing wool, which con-

sists in dyeing the material in a bath containing a dyestuff which is fast to stoving and sulfurous acid, all substantially as described.

2. The process of dyeing wool, which consists in dyeing the material in a bath containing rhodamin and sulfurous acid, all substantially as described.

In testimony whereof I have hereunto set my hand in the presence of two subscribing witnesses.

AUGUST SIEGMUND.

Witnesses:

BERNHARD C. HESSE,

JACOB ADRIAN.